

# UNITED STATES PATENT OFFICE.

LEE S. CHADWICK, OF EAST CLEVELAND, AND MARC RESEK, OF CLEVELAND HEIGHTS, OHIO, ASSIGNORS TO THE CLEVELAND METAL PRODUCTS COMPANY, OF CLEVELAND, OHIO, A CORPORATION OF OHIO.

## TREATMENT OF IRON OR STEEL FOR THE PREVENTION OF OXIDATION OR RUSTING.

1,320,734.

Specification of Letters Patent.

Patented Nov. 4, 1919.

No Drawing.

Application filed February 6, 1917. Serial No. 146,989.

To all whom it may concern:

Be it known that we, (1) LEE S. CHADWICK, (2) MARC RESEK, citizens of the United States, residing at (1) East Cleveland, (2) Cleveland Heights, in the county of Cuyahoga and State of Ohio, have invented a certain new and useful Improvement in the Treatment of Iron or Steel for the Prevention of Oxidation or Rusting, of which the following is a full, clear, and exact description.

This invention relates to improvements in the art of treating iron or steel articles, or articles having a coating of iron or steel, for the purpose of preventing the oxidation or rusting thereof, and wherein such articles are provided with a protective covering adapted to render the surfaces thereof capable of resisting, or of being unaffected by the action of, moisture and other oxidizing influences.

It has heretofore been proposed to treat iron or steel (or articles composed of or having a surface of iron or steel) with a dilute solution of ordinary phosphoric acid ( $H_3PO_4$ ) and preferably in the presence of iron filings or other compound intended to control or regulate the rapidity or strength of the chemical action upon the metal or articles undergoing treatment. It has been found that, in the practice of such process, it is necessary to boil the articles for a considerable length of time. Furthermore, the coating which is obtained upon the surfaces of the iron or steel articles is composed only of a mixture of normal ferric and ferrous phosphate.

We have found that, by boiling such articles in a bath containing a solution of the di-hydrogen phosphate of any metal (except the alkali metals) or by boiling such articles in a bath or solution containing chemicals in the proper proportion to form such a di-hydrogen phosphate, we are able to form upon the iron or steel surface a coating consisting essentially of a compound or mixture of normal phosphate of iron and a phosphate of the metal in solution, which coating is not only superior in its resisting qualities to any other so-called "rust-proof" coating with which we are acquainted but which coating can be formed upon the articles in a much shorter time than is required for the production of any other coat-

ing, for the purpose specified, with which we are acquainted. The metals employed for the production of such di-hydrogen phosphates are less basic than iron, which results in dissolving a certain amount of the iron and depositing upon the undissolved iron not only the compound or mixture of normal phosphate of iron and a phosphate of the metal in solution, but also a certain amount of the metallic constituent of the phosphate.

The bath employed by us may contain any normal phosphate of a metal less basic than iron or any mono-hydrogen phosphate, together with a sufficient quantity of an acid to furnish the necessary hydrogen to form a di-hydrogen phosphate and a sufficient quantity of any metallic compound to form the soluble di-hydrogen phosphate of that metal (except alkaline compounds, compounds of antimony, and mercuric chlorid). As nearly all metals form such soluble di-hydrogen phosphates, this necessarily includes compounds of nearly all metals except those mentioned.

One of the distinguishing features of our process is that in the practice of the same, no free phosphoric acid is present in the bath to which the iron or steel articles are subjected. In preparing such a bath, the following ingredients may be used:

Ordinary sodium phosphate, which is crystallized, di-sodium, mono-hydrogen phosphate;

Blue vitriol, or copper sulfate crystals;  
Sulfuric acid.

When these ingredients are mingled, the reaction which takes place is believed to be as follows:—



In actual practice, we have employed with good results 2,148 parts by weight of sodium phosphate crystals, with 1050 parts of blue vitriol crystals and 495 parts of 88% sulfuric acid to which sufficient water is added to form a standard solution. In practice we add to a tank containing about 500 gallons of boiling water a quantity of this solution that will contain about 14 lbs. of blue vitriol and a proportionate amount of each of the other ingredients. After treat-

- ing the articles for a period of, say 40 minutes, it will be found that, under ordinary conditions they are completely and satisfactorily coated. When it is desired to treat a 5 new batch of articles, the bath in the tank may be brought up to standard strength by adding thereto about one-sixteenth of the amount of the standard solution originally introduced.
- 10 In place of sodium phosphate, ammonium phosphate or any other alkali phosphate may be employed. Furthermore, in place of copper sulfate we may use manganese dioxid, zinc sulfate, aluminum chlorid, copper carbonate, or any other compound of a metal other than an alkali compound or compounds of a few metals, like barium, which do not form soluble phosphates. Furthermore, while any rather strong acid 15 (such as acetic, hydrochloric, or sulfuric) can be used, a nonvolatile acid, such as sulfuric, gives the best results, as in some cases a volatile acid will be given off by boiling the solution, requiring the addition 20 of a relatively large quantity of fresh acid to take the place of that which has been thus volatilized.
- 25 When the articles have been boiled in the bath consisting of the dilute solution described hereinbefore, the coating produced thereupon consists of a compound or mixture of normal phosphate of iron and the phosphate of the metal of the metallic salt in solution. In some cases this coating is 30 formed together with a coating of the metal of such salt.
- 35 It has been found in practice that mixtures of the following phosphates, metal salts, and acids work successfully in rust-proofing in accordance with our process:—

| <i>Phosphates.</i>  | <i>Metal salts.</i> | <i>Acids.</i>  |
|---------------------|---------------------|----------------|
| Sodium phosphate.   | Copper sulfate.     | Acetic acid.   |
| " "                 | " "                 | Sulfuric acid. |
| " "                 | Copper carbonate.   | Muriatic acid. |
| 45 " "              | Aluminum chlorid.   | Sulfuric acid. |
| " "                 | Manganese dioxid.   | " "            |
| " "                 | Zinc oxid.          | " "            |
| " "                 | Silver nitrate.     | " "            |
| Ammonium phosphate. | Iron sulfate.       | " "            |
| " "                 | Copper chlorid.     | " "            |

50 By employing a slight excess of the metallic salt over that required to form a di-hydrogen phosphate of metal, the coating formed upon the articles treated will, as indicated above, contain, in addition to the compound phosphate of iron and the metal 55 constituent of the salt, a coating of such metal constituent, additional to such phosphates, and which will be combined and embedded with such phosphate coating. Where copper sulfate is employed as the 60 metallic salt, the phosphate coating upon the iron or steel may have metallic copper deposited upon and embedded therewith, and this metallic copper will not only adhere firmly to the surface on which it is deposited, but will, by its presence, enhance 65

the rust-resisting qualities of such surface as well as impart thereto the capability of receiving special additional treatment, such as plating with copper or other metals. The proportion of copper sulfate appearing 70 in the formula hereinbefore set forth may be increased so as to furnish an excess of such metallic salt sufficient to secure the coating of metal (copper) upon the compound phosphate of iron and such metal 75 (copper). Where a coating of metallic copper is obtained, the presence of such coating will be manifest to the eye because of the reddish appearance thereof; and the amount of such coating may be varied by 80 suitably varying the excess of the copper sulfate over the amount set forth in the aforesaid formula, and this variation in the coating will be manifested by a like variation in the redness thereof.

Having thus described our invention, what we claim is:—

1. The process of treating iron or steel, or articles composed of or having a surface of iron or steel, which includes subjecting the 90 said article to the action of a bath made from a solution of an alkali phosphate and a salt of a metal less basic than iron, together with an acid.

2. The process of treating iron or steel, or 95 articles composed or having a surface of iron or steel, which includes subjecting the same to the action of a bath made from an aqueous solution of an alkali phosphate and a compound of a metal which will form a 100 soluble phosphate, together with sulfuric acid.

3. The process of treating iron or steel, or articles composed or having a surface of iron or steel, which includes subjecting the 105 same to the action of a bath containing the di-hydrogen phosphate of a metal less basic than iron and not containing free phosphoric acid or any oxidizing agent.

4. The process of treating iron or steel, or 110 articles composed of or having a surface of iron or steel, which includes subjecting the same to the action of a bath containing a solution of the di-hydrogen ortho-phosphate of a metal less basic than iron and not containing an oxidizing agent.

5. The process of treating iron or steel, or articles composed of or having a surface of iron or steel, which includes subjecting the same to a bath made from a solution of an 120 alkali phosphate together with sulfuric acid and a compound of a metal less basic than iron which will form a soluble phosphate.

6. The process of treating iron or steel, or articles composed of or having a surface of 125 iron or steel, which includes subjecting the same to the action of a bath containing a solution of the di-hydrogen phosphate of a metal less basic than iron.

7. The process of treating iron or steel, or 130

- articles composed of or having a surface of iron or steel, which includes subjecting the same to the action of a bath containing a solution of the di-hydrogen phosphate of a metal less basic than iron together with a small amount of another salt of such metal and which is capable of dissolving iron and depositing its metal constituent. 5 compound of a metal less basic than iron 25 which will form a soluble phosphate.
8. The process of treating iron or steel, or articles composed of or having a surface of iron or steel, which includes subjecting the same to the action of a bath containing a solution of copper di-hydrogen phosphate together with a small amount of copper sulfate. 10 11. Iron or steel, or articles composed of or having a surface of iron or steel, furnished with a coating containing iron phosphate combined with metallic copper. 30
12. Iron or steel, or articles composed of or having a surface of iron or steel, furnished with a coating containing a mixture of copper and iron phosphates combined with metallic copper. 35
13. Iron or steel, or articles composed of or having a surface of iron or steel, furnished with a coating containing a metallic phosphate combined with a metal less basic than iron. 40
9. In the treatment of iron or steel, or articles composed of or having a surface of iron or steel, subjecting such iron or steel to the action of copper di-hydrogen phosphate and copper sulfate. 20
10. A soluble compound for treating iron or steel, or articles composed of or having a surface of iron or steel, said compound containing an alkali phosphate, an acid, and a

In testimony whereof, we hereunto affix our signatures in the presence of two witnesses.

LEE S. CHADWICK.  
MARC RESEK.

Witnesses:

W. E. SHEPPARD,  
K. G. EAST.